# EUROPEAN PATENT APPLICATION

(11) **EP 1 369 504 A1**
(43) Date of publication of application: **10.12.2003**
(21) Application number: 02077255.4
(22) Date of filing: 05.06.2002
(51) Int. Cl.: C25D 15/00, C23C 18/16, H01R 13/03

(54) **Metal strip for the manufacture of components for electrical connectors**

(71) Applicant: Hille & Müller, D-40589 Düsseldorf (DE)
(72) Inventor: Holtkamp, Johannes Henricus Maria, 40724 Hilden (DE); Giesler, Martin, 40764 Langenfeld (DE); Celis, Jean-Pierre Paul Julien Clement Frans, 3360 Korbeek-Lo (BE)
(74) Representative: Hansen, Willem Joseph Maria

(57) **Abstract**

Metal strip for the manufacture of components for electrical connectors comprising a metallic core and a galvanically deposited metal containing coating layer, whereby the metal containing coating layer is deposited by electrolytic or electroless composite plating and the coating layer comprises a metal matrix and distributed therein particles selected from the group of particles having electrically conductive properties, particles having lubricating properties, particles having wear resistance properties and particles having properties of increasing the temperature durability or combinations of particles from those groups.

## Description

The invention relates to a metal strip for the manufacture of components for electrical connectors comprising a metallic core and a galvanically deposited metal containing composite coating layer.

The invention also relates to a method for the manufacture of such strip, an electrical connector comprising such metal strip and to the use of such metal strip for the manufacture of an electrical connector.

In connection with the present application an electrical connector is to be understood as any means for making an electrical connection between two parts, such as but not limited to temporarily, permanently, by hand, by mechanical or electrical force, in single or multiple form.

A metal strip for use in electrical connectors is known from EP 0 849 373 A1. That publication discloses a metal strip from copper, iron, nickel, zinc or its alloys as metallic core which is coated with a coating layer mainly consisting of tin or tin alloy. In the most outer skin of the coating layer, 1 to 50 atomic weight percent of carbon is incorporated. The purpose of the incorporation of carbon is to obtain an improved wear- and corrosion behaviour, in particular fretting corrosion, while at the same time having an oxide free surface.

That method for making the metal strip comprises applying a tin coating layer by hot dip tinning or electrolytic tin-plating into the metallic core. Subsequently, the metallic core with the tin coating layer is fed through an oil bath at elevated temperature above the melting point of the tin or the tin alloy to incorporate carbon in the tin coating layer. Preferably, to obtain a higher carbon content, the metal strip is cooled in a second oil bath.

A problem with the known method is that at least one additional process step after applying the coating layer is required.

Another problem is that the method can only be applied to coating layer metals of relatively low melting points.

A further problem is that only carbon can be incorporated as the component to improve the desired characteristics of the metal strip as starting material for electrical connectors.

However, carbon only provides a solution for some, but not all requirements of electrical connections. So, the proposed method is only applicable for a limited number of applications of electrical connectors.

It is an object of the present invention to provide a metal strip for the manufacture of components for electrical connectors with a large amount of particles in the coating layer, preferably all throughout the coating layer.

It is a further object of the present invention to provide a metal strip for the manufacture of components for electrical connectors in which the coating layer has properties that are optimally adapted to the intended use of the electrical connectors.

It is yet another object of the present invention to provide a metal strip for the manufacture of components for electrical connectors that can be manufactured in a single process step.

It is a further object of the present invention to provide a metal strip for the manufacture of components for electrical connectors which gives more freedom in the selection of the metal matrix of the coating layer and of the particles embedded therein.

These and other advantages are obtained with a metal strip for the manufacture of components for electrical connectors which according to the invention is characterized in that the metal containing coating layer is deposited by electrolytic or electroless composite plating. That coating layer comprises a metal matrix and distributed therein particles selected from the group of particles having electrically conductive properties, particles having lubricating properties, particles having wear resistance properties, and particles having properties of increasing temperature stability or combinations of particles from those groups. This process is also referred to as co-deposition in this application.

Patent publication 5,028,492 relates to a composite coating for connectors. The composite coating comprises a ductile metal matrix of a selected composition and a uniformly dispersed polymer component. In one embodiment of a method of applying the composite coating it is proposed to deposit the coating directly on a connector in an electroless or electrolytic plating process.

According to the present invention the metal containing coating layer is deposited on an essentially flat metal strip, plate or sheet. This brings the advantage of good controllability of the co-deposition process, a good uniformity of the thickness of the coating layer and a good homogeneity of the distribution of the particles within the coating layer, because side-effects are eliminated and nonuniform distribution of the electrical field is prevented.

For certain compositions the electroless plating process can be applied. This process has the advantage that it does not require an external electrical potential and contact to the metallic core during processing. The electrolytic process has the advantage of good controllability of the process in particular with regard to thickness and uniformity of the coating layer and can be applied to a wide range of coating layer compositions.

There are, depending on the application, several requirements an electrical connector should fulfil. A first requirement is a low electrical resistance. The electrical resistance may increase over time due to corrosion of the outermost layer of the material of which the contacts of the connector are manufactured.

Also effects, known as tribo-oxidation or fretting may occur. In case the electrical connectors are used in a vibrating environment, closed contacts may move slightly in a tangential direction, relative to each other, thereby disrupting a formed oxide layer that can act as an abrasive, exposing non-oxydised contact material to the atmosphere. The abraded particles may deposit between the closed contacts, thereby increasing the contact resistance.

A relative movement of the closed contacts may also be caused through thermal expansion of the used materials. Through changes of the environmental temperatures or as a consequence of heat generation caused by the current passing through closed contacts, the connector may change in temperature causing relative movement of the closed contacts. This may also lead to tribo-oxidation.

Another important characteristic of a connector is the insertion force needed to insert a first part of a connector into the co-operating second part of the connector. Related hereto is the extraction force needed to disengage a connector.

The metal strip according to the invention can be given the selected, optimum characteristics in dependence of the selection of the particles embedded in the coating layer. The most important characteristics being low contact resistance, low oxidation, high corrosion resistance, low tribo-oxidation or fretting, low insertion and extraction forces.

By selecting particles having high electrical conductivity a low contact resistance can be obtained. The low contact resistance is maintained even when the metal of the metal matrix oxidises at its surface, in particular in the event the particles protrude from the metal matrix.

By selecting particles having lubricating properties, a low insertion and/or extraction force can be obtained when the particles protrude from the metal matrix. An additional advantage is that fretting is also reduced.

By selecting particles having high wear resistance properties it is achieved that under vibrating conditions or in applications requiring frequent insertions and extractions, contact wear is reduced. Consequently, fewer particles are rubbed off and built up between the contacts. This has the effect that the contact resistance increases less over time and/or use.

By selecting particles having heat resistance and conductive properties it is achieved that under high temperature conditions, the contact resistance remains low and/or corrosion or oxidation is low, i.e. the characteristics of the electrical connector are less temperature and time dependent. The particles having conductive properties will make sure that the conductivity stays low, even if part or all of the coating layer oxidises.

Preferred embodiments of the invention are given in the dependent claims.

The selection of the metal of the metal matrix can be based on the purpose for which the electrical connector is used and the conditions of use.

The metal used for the metal core can be selected from a wide range of metals, also dependent on the purpose for which the electrical connector is used and the conditions of use.

By co-depositing the metal of the metal matrix and the particles, it is possible to select the size of the particles within a broad range, such as between 0,001 µm and 15 µm, dependent on the composition of the particles and their purpose in the coating layer. Size is to be interpreted as the diameter of the smallest sphere enclosing a particle.

This co-depositing also makes it possible to embed a broad range of volume fractions of the distributed particles in the coating layer, again dependent on the requirements during operation or the lifetime of the electrical connector.

Since the process of co-depositing on a flat strip, sheet or plate is very well controllable, the thickness of the coating layer can be matched very well to the requirements put on the connectors. Coating layers in the range of 0,2 - 10 µm are preferred. Thinner layers in general do not meet the requirements; for thicker layers alternative processes could be considered in view of the time required for the co-deposition of the metal matrix and the distributed particles makes it possible to homogeneously distribute the particles in thickness direction within the coating layer. The coating layer, therefore, also has uniform characteristics over the thickness and the total coating layer does not need to be thicker than required for normal operation during the lifetime of the connector or the apparatus in which the connector is used.

The invention is also embodied in a method for the manufacture of components for electrical connectors, wherein a metallic core is fed through a galvanic bath and a coating layer is deposited on at least one side of the metallic core.

Such method is know from EP 0 849 373. A drawback of the prior art method is that this method is only applicable for a metal matrix of tin or its alloys in which an outer carbon containing layer is deposited. Furthermore, the method requires at least two steps: one step for applying the metal matrix and a second step for depositing the carbon containing layer.

An object of the invention is to provide a method with which it is possible to deposit the coating layer in one single step and which method provides a great flexibility in the choice of the metallic core, and the composition of the coating layer.

These objects and other advantages are obtained with a method which is, according to the invention, characterized in that a metal matrix and particles selected from the group of particles having electrically conductive properties, particles having lubricating properties, particles having wear resistance properties or particles having properties of increasing the temperature durability and combinations thereof, are deposited on the metal core to form the coating layer.

The method makes it possible to apply in one single process step a metal matrix and distribution therein particles which can be selected from a wide range of materials, dependent on the desired characteristics of the composite coating layer.

## Claims

1. Metal strip for the manufacture of components for electrical connectors comprising a metallic core and a galvanically deposited metal containing coating layer, **characterized in that** the metal containing coating layer is deposited by electrolytic or electroless composite plating and the coating layer comprises a metal matrix and distributed therein particles selected from the group of particles having electrically conductive properties, particles having lubricating properties, particles having wear resistance properties and particles having properties of increasing the temperature durability or combinations of particles from those groups.

2. Metal strip according to claim 1, **characterized in that** the electrically conductive particles are selected from the group comprising carbonaceous materials such as soot, graphite, carbonaceous nanotubes: electrically conductive ceramic materials comprising borides, such as titanium boride and iron boride; nitrides such as titanium nitride and chromium nitride; sulfides such as titanium sulfide, tantalium dissulfide and molybdeen dissulfide and electrically conductive oxides such as titanium oxide.

3. Metal strip according to claim 1 or 2, **characterized in that** the particles having lubricating properties are selected from the group comprising polymers, such as PTFE, polyimide and polyamide; carbon containing particles such as essentially pure carbon, graphite, ceramic particles such as molybdeen disulphide and borium nitride and lubricating means containing capsules such as capsules containing polyphenylether or organic lubricating means and optionally the particles having lubricating properties also having corrosion inhibiting additives.

4. Metal strip according to any of the preceding claims, **characterized in that** the particles having wear resistance properties are selected from the group comprising ceramic particles such as aluminium oxide, zirconium oxide, silicon carbide, boron nitride and titanium nitride.

5. Metal strip according to any of the preceding claims, **characterized in that** the particles having properties of increasing temperature durability are selected from the group comprising heat resistant and conductive ceramic particles such as aluminium oxide, zirconium oxide, silicon carbide, diamond-like boron nitride and titanium nitride.

6. Metal strip according to any of the preceding claims, **characterized in that** the co-deposited metallic matrix mainly comprises one or more metals selected from the group nickel, copper, tin, zinc, chromium and alloys or combinations thereof.

7. Metal strip according to any of the preceding claims, **characterized in that** the metallic layer mainly comprises one or more metals selected from the group low carbon steel, high-strength steel, stainless steel, copper, including bronze and brass and multilayer composites alloys or mixtures thereof.

8. Metal strip according to any of the preceding claims, **characterized in that** the distributed particles have a size in the range of 0.001 - 15 µm.

9. Metal strip according to any of the preceding claims, **characterized in that** the volume fraction of the distributed particles in the co-deposited coating layer is in the range of 0.7% to 30% of the volume of the coating layer.

10. Metal strip according to any of the preceding claims, **characterized in that** the thickness of the metal strip is in the range of 0.1 to 1.5 mm.

11. Metal strip according to any of the preceding claims, **characterized in that** the coating layer has a thickness in the range from 0.2 - 10 µm.

12. Metal strip according to any of the preceding claims, **characterized in that** the particles of at least one group, preferably of all groups of particles, are homogeneously distributed in the coating layer.

13. Method for the manufacture of a metal strip according to any of the claims 1 to 12 for use for the manufacture of components for electrical connectors, wherein a metallic core is fed through a galvanic bath and a coating layer is deposited on at least one side of the metallic core, **characterized in that** a metal matrix and particles selected from the group of particles having electrically conductive properties, particles having lubricating properties, particles having wear resistance properties or particles having properties of increasing temperature stability and combinations thereof, are co-deposited on the metal core to form the coating layer.

14. Method according to claim 13, **characterized in that** the method is performed in a continuous or semi-continuous manner.

15. Electrical connector or electrical switching element comprising at least one part thereof manufactured from a metal strip according to any of the claims 1-12.

16. Use of a metal strip according to any of the claims 1-12 in the manufacture of an electrical connector or electrical switching element.
